

## UNITED STATES PATENT OFFICE.

FRANCIS DAVID CORBIN, OF LLANELLY, CARMARTHEN, SOUTH WALES, ASSIGNOR OF THREE-EIGHTHES TO THE LLANELLY FOUNDRY & ENGINEERING COMPANY LIMITED AND ONE-THIRD TO RICHARD NEVILLE & COMPANY LIMITED, BOTH OF LLANELLY, CARMARTHEN, SOUTH WALES, GREAT BRITAIN.

## ROLL FOR ROLLING METALS AND METHOD OF MAKING SAME.

No Drawing. Application filed June 28, 1927, Serial No. 202,756, and in Great Britain July 7, 1926.

This invention relates to improved rolls for rolling metals.

Quenched rolls have the disadvantage that enormous internal stresses are generated on quenching, while hair-cracks and similar surface flaws are liable to develop in the working surface, these defects causing "spalls" during the working of the roll. In chilled cast iron rolls, which are brittle and have poor mechanical strength throughout, the chilled iron rim or "chill" has a rate of expansion under heat which is twice that of the grey iron core, so that enormous internal stresses are set up on increase of temperature. Great internal stresses are also set up when the roll is cast, owing to the rapid cooling of the roll body, and, moreover, when the chill is worn out it cannot be renewed. A further common disadvantage of quenched and chilled rolls is the difficulty in manufacturing them for rolling complicated sections.

The object of this invention is to obviate these disadvantages and to provide rolls for rolling metals having higher physical properties than the rolls at present in general use and which may be manufactured in complicated shapes.

According to the present invention I provide a roll for rolling metals, made in case-hardened alloy steel and having its case-hardened portion of a hard "martensitic" "troostitic", "cementitic" or allied structure and its remaining portion of a soft "pearlitic" or allied structure, both structures being obtained with the same slow rate of cooling from high temperatures, that is to say, such rate of cooling as may be obtained without external aids, such as immersion in, or spraying with, any liquid. To this end, certain elements, such for example, as nickel or manganese, are introduced into the steel, and which, in the presence of sufficient carbon, tend to retain the metal in the hard martensitic, troostitic, cementitic or allied condition, after a rate of cooling so slow that a steel of the same carbon content, but without said elements, would have passed into the relatively soft pearlitic condition. In these alloys, the effect of carbon on this tendency, for a given proportion of the special element, or elements is cumulative, that is, a suitably chosen alloy will be pearlitic, soft and tough, with a low percentage of carbon, but troostitic, martensitic, cementitic or of

allied structure and very hard, with a high percentage of carbon, on being cooled slowly in both cases.

Having selected the constituents for the steel alloy which will give, for each individual case, suitable physical characteristics in the core of the roll with a low percentage of carbon, and suitable physical characteristics combined with great hardness on the working face with a high percentage of carbon, I then make the roll of an alloy containing a low percentage of carbon and such amounts of the other constituents as will give, on slow cooling, with this low percentage of carbon, a pearlitic or allied structure, and with a suitable high percentage of carbon, to be introduced into the case by case-carburizing a martensitic, troostitic, cementitic or allied structure, as may be required, thus attaining maximum hardness for the case without the necessity for reducing the temperature of the roll from high temperatures in water or other liquid, with all the risks attendant on this procedure.

Of the elements which may be usefully employed for alloying in the process, manganese, vanadium, tungsten, chromium and molybdenum, favour the absorption of carbon by solid steel during case-hardening, while nickel tends to hinder it where solid case-hardening cements are used. Thus, if nickel is used in conjunction with a solid cement, one or more of the first mentioned elements should be used with it to counteract this tendency, while this addition of a further special element or elements can generally also by careful choice be made to enhance the general qualities of the resultant alloy. Nickel and chromium, for example, form a very suitable combination for many purposes.

By way of example, I will describe the making of a roll, for cold rolling of metals, in a nickel-chrome steel alloy. For hardness without unnecessary brittleness, the case should be at, or slightly above, the eutectoid composition, say, 1.0 per cent carbon. For normal cooling in air, with 1.0 per cent carbon, 5.0 per cent nickel will give a martensitic structure, but with carbon contents appreciably below 0.80 per cent the structure will be pearlitic. For a nickel content of 5.0 per cent 0.80 per cent of chromium will be sufficient to ensure carbon absorbing prop-

erties with solid cements, and will give a harder case without unduly increasing brittleness while, further, the structure will not coarsen under heat treatment in the presence of so much nickel.

I cast or forge the roll in a steel containing approximately

|    | Ni.  | Cr.   | C     |
|----|------|-------|-------|
| 10 | 5.0% | 0.80% | 0.20% |

The roll is then well annealed and is allowed to cool to room temperature and then machined, the body being brought to a smooth finish and left, say, .015" overall full to final size. After machining, the roll is case carburized in a box having removable ends, or other device, to allow of its rapid removal whilst hot.

With the carburizing mixture consisting of 20 60 per cent oak, or beech, charcoal and 40 per cent barium carbonate, a temperature of 900° C. will give approximately 1.0 per cent carbon in the case for this composition, the time taken obviously varying with the depth 25 of case required and being easily determined. (Where very deep cases are required, it is preferable to use pure charcoal at higher temperatures, reducing the nickel and the chromium contents to correspond with the higher 30 carbon percentage thus obtained in the case.)

At the conclusion of the carburizing procedure, the grain structure of the core may be refined by allowing the roll to cool down in its carburizing box to well below the thermal 35 critical range of the core material, whereafter it is reheated to approximately 100° C. above said range, and after being kept at this temperature for a sufficient time to ensure that the structure shall have passed into the 40 solid solution condition, the roll in its box is removed from the furnace. On removal from the furnace, the roll is stripped, and allowed to cool in air. Where an exceptionally tough core is required the refining process 45 may be doubled, that is to say, the roll after its preliminary cooling from the case-hardening temperature may be first reheated up to, and furnace cooled from, above the critical range of the core, then re-heated up 50 to just below the said critical range and cooled in air.

When no grain structure refining procedure is utilized, the roll will be removed from the furnace at the lowest temperature from 55 which air cooling will give the required degree of hardness in the case.

After cooling, the roll is finally ground to size and polished, the machining allowance given above being sufficient for the removal of any slight decarburized "bark" (that is, the extremely thin skin of metal which is robbed of its carbon by oxidation during the final cooling down in air).

It should be noted that when the final cooling of the roll in air is for any reason un-

desirable, or when either extreme hardness on the working face of the roll is unnecessary or a composition may be used which, with the amount of carbon to be introduced by case-hardening in the particular instance, will be so far removed from the structure-transition range as to ensure that, even on very slow cooling, the case structure will remain in the required hard condition, the final cooling of the roll, may take place in the carburizing box either in or out of the furnace and not in air. In this case, the case-hardening material packed around the roll in the carburizing box is not disturbed.

I claim:

1. A roll for rolling metals, made in case-hardened alloy steel and having its case-hardened portion of a hard structure, and the remaining portion of a soft pearlitic or allied structure, both structures being obtained with the same slow rate of cooling of the roll from high temperatures.

2. A roll as claimed in claim 1, containing one or more of the elements manganese, vanadium, tungsten, chromium, or molybdenum as constituents in the steel alloy.

3. A roll as claimed in claim 1, containing the element nickel as a constituent in the steel alloy, and one or more of the elements manganese, vanadium, tungsten, chromium or molybdenum.

4. A roll as claimed in claim 1 having an interior with a low carbon content and having a high percentage of carbon in the case.

5. A method of making a roll for rolling metals, which consists in providing an alloy steel containing approximately

|    | Ni.  | Cr.   | C     |
|----|------|-------|-------|
| 10 | 5.0% | 0.80% | 0.20% |

forming a roll therefrom, annealing the product, cooling it, machining the cooled product, case-hardening it, allowing it to cool to below the thermal critical range of the core, reheating to about 100° C. above said range 110 keeping it at this temperature for a sufficient time to ensure that the structure shall have passed into the solid solution condition, and allowing the roll to cool.

6. A method of making a roll for rolling metals, which has the steps of subjecting an alloy steel to case-hardening in the presence of a high temperature, and then cooling at a slow rate both the case and the interior, such slow rate of cooling being the same for 120 both and a rate that produces a hard case and a soft core.

7. A method of making a roll for rolling metals, which has the steps of providing an alloy steel with a low percentage of carbon, and with a constituent that on slow cooling from a high temperature will give a soft, pearlitic or allied structure, increasing the carbon content by the application of a high temperature, and then cooling at a slow rate 130

both the carburized exterior, such rate being one that produces a hard case and a soft core.

8. A method of making a roll for rolling metals, which has the steps of subjecting an alloy steel to case-hardening in the presence of a high temperature, and then cooling at a slow rate both the case and the interior; such slow rate of cooling being the

same for both and a rate that produces a hard case and a soft core, reheating the roll to the critical range of the core, furnace-cooling it, again reheating short of said critical range, and then cooling.

In testimony whereof I have signed this 15 specification.

FRANCIS DAVID CORBIN.